

84 -M

Patented May 10, 1932

1,857,201

## UNITED STATES PATENT OFFICE

HUBBEL LATHROP, OF GREENWICH, CONNECTICUT, ASSIGNOR TO BELL TELEPHONE LABORATORIES, INCORPORATED, OF NEW YORK, N. Y., A CORPORATION OF NEW YORK

## PROCESS FOR INSULATING MAGNETIC BODIES

No Drawing.

Application filed July 2, 1931. Serial No. 548,484.

This invention relates to magnetic bodies and particularly to methods of producing magnetic bodies of the type employing finely divided magnetic material.

5 An object of the invention is to improve the magnetic characteristics of magnetic bodies of the type employing magnetic material in finely divided form, for example, magnetic dust cores for loading coils.

10 Magnetic cores made from finely divided magnetic material, so-called magnetic dust cores, are being extensively used for the loading coils which are inserted in telephone lines to improve their transmission characteristics.

15 Such cores are usually constructed by subjecting the finely divided particles of the magnetic material and a non-magnetic material between the magnetic particles, to extremely high pressures in the neighborhood 20 of 200,000 pounds per square inch. The high pressures are utilized to form the component materials into a substantially homogeneous mass in the desired core form, and to give sufficient mechanical strength to the completed

25 core. The non-magnetic material is of such a nature as to serve as a binder, and also as an insulation between the magnetic particles to reduce eddy current losses in the completed core. In the case especially where the mag-

30 netic material in the core made in the above described manner is a magnetic alloy including nickel and iron, it is desirable also to subject the core to subsequent heat treatment at a high temperature to remove the strains in-

35 introduced in the magnetic material by the pressing operation tending to impair the magnetic properties of the magnetic alloy in the core, and to fully develop the magnetic characteristics of the alloy. It is desirable,

40 therefore, that the insulating material have such characteristics and be applied in such manner to the dust particles that it will withstand without deterioration from an insulating standpoint the heat treatment and mechanical operations utilized in producing the core.

A method commonly used for insulating the magnetic dust in the process of making loading coil cores is to mix the magnetic dust with the insulating material in finely divided

form, and a volatile liquid, such as water, and then to evaporate the whole to dryness with constant stirring in order to coat the magnetic particles with the insulating material. The total amount of insulating material 55 is thus applied to the magnetic dust particles in one layer. The insulated magnetic particles are then compressed under high pressure into the desired core form, and the resulting cores are given a subsequent annealing heat treatment to improve their magnetic characteristics.

In accordance with the present invention the process of insulation above described is modified in that the insulating material is applied to the magnetic dust particles a portion 60 at a time so as to obtain several layers of the same insulating material between the magnetic particles. This change in the method of insulating has been found to materially 65 improve the magnetic properties, and particularly to reduce the eddy current loss in the completed core.

The exact nature of the invention and the advantages thereof will be better understood 70 from the following detailed description of the process for producing a magnetic dust core or a loading coil embodying the invention.

In practicing the present invention, the magnetic material is preferably prepared from a brittle alloy containing nickel and iron, with or without the addition of other constituents, and commonly known as "perm-alloy". The alloy may be prepared in the 75 manner described in the U. S. Patent No. 1,669,649 issued May 15, 1928 to C. P. Beath and H. M. E. Heinicke, wherein the magnetic metals, for example, nickel and iron in proportions depending upon the desired percentage of the alloy, are melted together in an oxidizing atmosphere, the resulting alloy being poured into a mold to form an ingot. The ingot while still hot is successively passed 80 through progressively reducing rolls to decrease its cross-section, the final roll being 85 preferably effected at approximately the temperature at which the alloy ceases to be malleable, after which the ingot is quenched in water 90 at a temperature below that in which it loses 95 100

its malleability. This treatment is for the purpose of producing a fine crystalline structure in the alloy material since when the material is reduced to finely divided form its dis-  
5 integration takes place at the crystal bound-  
aries, and consequently the smaller the size  
of the crystals the finer the dust which can  
be produced therefrom. The slabs of alloy  
material so produced are then broken into  
10 short pieces and the pieces reduced to the form  
of dust in any suitable manner for example  
by crushing in a rock crusher, hammer mill,  
or other suitable apparatus, after which the  
crushed material is pulverized by rolling in  
15 a ball mill for several hours. After several  
hours of rolling the resulting dust is sieved  
through a 120 mesh sieve and that portion  
which will not pass through the sieve is re-  
turned to the ball mill for further rolling,  
20 this process being repeated until a sufficient  
quantity of the very fine dust is obtained.  
Prior to the addition of the insulating mate-  
rial the finely divided particles of the alloy  
are annealed in a closed container at a tem-  
25 perature of approximately 885° C. It is then  
necessary to again reduce the annealed alloy  
which is now in the form of a cake to a finely  
divided form ready for insulation.

The general method of insulating the mag-  
30 netic particles in accordance with this inven-  
tion was tried with several insulating com-  
positions. In each case a material improve-  
ment in the magnetic properties of the com-  
pleted core was observed over that obtained  
35 when the usual method of insulation was em-  
ployed.

In one case the method of the invention was  
applied to the insulation of the annealed mag-  
30 netic particles with an insulating composi-  
tion comprising kaolin, talc, sodium silicate,  
chromic acetate and water, such as disclosed  
and specifically claimed in my copending ap-  
plication, Serial No. 556,951, filed August 14,  
1931. It was desired to insulate 1000 grams  
45 of the annealed permalloy dust with a total  
of 6.5 grams finely divided kaolin, 6.5 grams  
finely divided talc and 11.0 grams of sodium  
silicate in solution with 1.1 grams of chromic  
acetate.

50 This was done as follows:

The 11.0 grams of sodium silicate and 1.1  
grams of chromic acetate were first dissolved  
in water to a total solution volume of 333 cc.  
Each 1000 grams of permalloy dust were then  
55 mixed with 2.5 grams finely divided talc and  
2.5 grams finely divided kaolin, 111 cc. of  
the solution of sodium silicate and chromic  
acetate was added thereto and then the mix-  
ture was evaporated to dryness with constant  
60 stirring, to form the first layer of the insula-  
tion on the permalloy dust particles.  
Then, an additional 2.0 grams talc and 2.0  
grams kaolin were mixed with the coated  
65 magnetic particles, an additional 111 cc. of  
the solution added thereto, and the whole

evaporated again to dryness with constant  
stirring, to form a second layer of insulation  
on the permalloy dust particles. Then the  
resulting coated magnetic particles were  
mixed with the remaining 2.0 grams talc and  
2.0 grams kaolin, the remaining 111 cc. of  
the solution added thereto, and the whole  
evaporated to dryness to form a third layer  
of insulation on the magnetic particles.

In another case it was desired to insulate  
the annealed permalloy dust with an insu-  
lating composition such as disclosed in my  
copending application, Serial No. 459,564  
filed June 6, 1930. The insulating material  
used comprises 1.6 grams sodium silicate and  
1.0 grams talc for each 100 grams of the  
magnetic dust. A solution of the sodium  
silicate in water was first made up, 40 cc. of  
water being used for each 1.6 grams of the  
sodium silicate. One third of the talc in  
dry powder form was then mixed with the  
total amount of the permalloy dust, one third  
of the sodium silicate solution was added  
thereto, and then the whole evaporated to  
dryness to form the first insulating layer on  
the magnetic particles. The insulated mag-  
netic particles were then mixed with another  
one third of the talc, another one third of  
the sodium silicate solution was added there-  
to and the resulting mixture was again evap-  
orated to dryness to form the second coating  
of the insulating material on the magnetic  
dust particles. The remaining one third  
portion of talc was then mixed with the insu-  
lated magnetic dust particles, the remaining  
one third of the sodium silicate solution was  
added thereto and then the resulting mixture  
was evaporated to dryness to form the third  
coating of insulating material upon the mag-  
netic particles.

The magnetic dust particles insulated with  
the different insulating compositions in the  
above described manner were respectively  
sifted through a 16 mesh sieve, placed in a  
mold and compressed into core parts under  
a pressure of approximately 200,000 pounds  
per square inch. The core parts were then  
transferred to an annealing furnace where  
they were annealed at a high temperature  
either in air or in hydrogen to relieve the  
internal stresses set up by the pressing opera-  
tion, thereby producing a core having low  
hysteresis loss.

Where the annealing heat treatment is  
carried out in air, the core parts are prefer-  
ably subjected to a temperature of approxi-  
mately 500° C. for about 45 minutes. Where  
the annealing heat treatment is carried out  
in hydrogen, the core parts are preferably  
subjected to a temperature of approximately  
650° C. for about 30 minutes.

One or more core parts thus formed are  
then stacked to form a core to which the us-  
ual toroidal winding is applied to form a  
loading coil, the number of core parts used in

each core depending upon the electrical characteristics of the circuit with which the loading coil is to be associated.

Tests of magnetic cores insulated by the method of the invention in which the insulating material was applied in three or more stages as described above and other cores made at the same time using the same amount and kind of insulating material applied in a single layer by the usual method, showed that the former method resulted in much lower eddy current losses in all cases and in most cases in improved hysteresis characteristics as well. In the case of the particular insulating materials mentioned above, the reduction in eddy current losses obtained by the method of the invention was found to be approximately 20 to 60 per cent lower than that obtainable employing the methods of the prior art.

It is to be understood that the invention is not limited to the particular constituents and proportions of the magnetic and insulating materials above mentioned which were given by way of example only, but that it is of a generic nature applicable to all magnetic and insulating materials which are commonly used in the production of magnetic bodies of the type employing magnetic material in finely divided form. It is to be understood also that the method of applying the insulating material may be varied somewhat from that described above without departing from the spirit of the invention which is limited only within the scope of the appended claims.

What is claimed is:

1. In the process of making a magnetic body comprising finely divided magnetic particles insulated from each other by a given amount of insulating material, the method of insulating the magnetic particles which consists in mixing said particles with a portion of the insulating material in a volatile liquid and evaporating the mixture to dryness, and mixing the resulting product with another portion of the insulating material in a volatile liquid and evaporating to dryness.

2. In the process of making a magnetic body comprising finely divided magnetic particles insulated from each other by a given amount of insulating material, the method of insulating the magnetic particles which consists in mixing said magnetic particles with a portion of the total amount of insulating material in a volatile liquid and evaporating the mixture to dryness to form an insulating coating on the particles, mixing the coated particles with another portion of the insulating material in a volatile liquid and evaporating the mixture to dryness to form a second layer of insulating material on the particles, and repeating the process until the entire amount of insulating material has been applied to the magnetic particles in layers.

3. The method of producing a magnetic

body having a low eddy current loss from a given amount of finely divided magnetic material and a given amount of a finely divided insulating and binding material including both soluble and insoluble ingredients, which method consists in mixing the total amount of the magnetic material with a portion of the insoluble ingredients of the insulating and binding material in dry form, adding to the mixture a liquid solution of a portion of the soluble ingredients of the insulating and binding material and evaporating the whole to dryness with constant stirring, mixing the resulting coated magnetic particles with another portion of said insoluble ingredients in dry form; adding to the resulting mixture a liquid solution of another portion of said soluble ingredients and evaporating the whole to dryness with constant stirring, repeating the process until all of the insulating and binding material has been applied as coatings to the magnetic particles, compressing the resultant product into a substantially homogeneous mass in the desired form, and then heat treating the formed product to remove strains in the magnetic material.

4. In the process of making a magnetic body comprising finely divided particles of magnetic material insulated from each other by a given amount of insulation comprising several constituent materials, the method of insulating the magnetic particles which consists in mixing in a volatile liquid said magnetic particles with a portion of the insulation comprising a portion of each of the constituent materials and evaporating the mixture to dryness, mixing the resulting product in a volatile liquid with another portion of the insulation comprising a portion of each constituent material and evaporating the mixture to dryness, and repeating this process until the entire amount of the insulation has been applied to the magnetic particles in successive layers.

In witness whereof, I hereunto subscribe my name this 1st day of July, 1931.

HUBBEL LATHROP.

115

120

125

130